

## UNITED STATES PATENT OFFICE

2,149,480

## PROCESS OF MANUFACTURING PIG IRON

Max Paschke, Clausthal-Zellerfeld, and Eugen Peetz, Duisburg-Hüttenheim, Dusseldorf, Germany, assignors to H. A. Brassert & Company, Chicago, Ill., a corporation of Illinois

No Drawing. Application October 1, 1937, Serial No. 166,718. In Germany April 15, 1936

4 Claims. (Cl. 75—41)

This invention relates to a new and improved process for the manufacture of pig iron low in sulphur and more particularly to a process in which the desulphurization is carried out, in part at least, in the lower portion of the blast furnace.

Previously, processes for the manufacture of pig iron in the blast furnace, from a burden rich in particular in silica, or sulphur, and using coke more or less high in sulphur, have been developed, in which fluxes, such as limestone, are added to the burden only in such quantities that a high-sulphur iron is produced, together with an acid slag of low-melting point, the iron after tapping being desulphurized by means of a basic slag, or other usual means.

According to this prior process the smelting of silicious low-grade ores, which is normally uneconomical, becomes possible in that desulphurization in the blast furnace is dispensed with, and only sufficient limestone is added to the burden to obtain an easily fusible acid slag, for instance of the type obtained from a charcoal furnace. By this means a large reduction in coke consumption is obtained when smelting low-grade silicious ores, because among other things, the yield per unit of burden is considerably increased, and the fuel consumption in the blast furnace, when using easily fusible acid slags, is largely reduced. In comparison with operations using slags of the usual basicity, which, however, effect complete desulphurization of the iron in the blast furnace.

It is an object of the present process to provide a method for economically obtaining iron low in sulphur.

It is a further object to provide a method whereby a portion at least of the sulphur is removed in the lower portion of a blast furnace.

It is also an object to provide a method whereby desulphurizing reagents may be supplied directly to the lower blast furnace zones.

Other and further objects will appear as the description proceeds.

In accordance with the present invention, prior processes are extended and improved by carrying out some of the desulphurization in the lower part of the blast furnace, rather than entirely outside the furnace, without, however, sacrificing the advantages obtained. The burdening of the furnace is similar to that proposed in the above described process, i. e., the low-grade and silicious iron ores have only enough fluxes, such as limestone, added in order to form an easily fusible acid slag. In the lower part of the blast furnace, preferably below the bosh, desulphurizing agents

are blown into the charge, which to a large extent is reduced, or even melted. In this way a considerable quantity of sulphur can be removed from the iron without having to charge the desulphurizing agents originally with the ore and coke.

It is advantageous to blow in the desulphurizing agents, such as limestone, soda, fluorspar, manganese, in the form of ore, slag, ferro-manganese, and so forth, at such a position, low down in the blast furnace, that they will act as effectively as possible directly on the pig-iron bath beneath the tuyères.

In order to obtain the full advantages from smelting with a silicious and free-running slag, and to avoid blowing into the blast furnace more than a minimum of the desulphurizing agents, it has proved advantageous to effect the blowing in of the desulphurizing agents intermittently.

This intermittent process is carried out according to one form as follows:

After a certain quantity of pig iron and acid slag has collected in the blast-furnace hearth, i. e., a short time before tapping, the free-running acid slag is removed from the high-sulphur iron. The desulphurizing agents are then blown in on the practically slag-free pig iron, or on the charge in its proximity, and after a short period the slag so formed is withdrawn from the pig iron, or this slag is tapped, together with the iron, in a known manner. The sulphur content of the pig iron, subjected in this way to a preliminary desulphurization, can if necessary be further reduced outside the blast furnace.

The blowing in of material to be smelted is in itself known. The present improvement of the prior processes makes possible the smelting of highly silicious low-grade iron ores in the blast furnace to produce pig iron comparatively low in sulphur, retaining the advantages of the prior process, and obtaining economy of operation in that the cost of desulphurization outside of the blast furnace is saved.

The apparatus for blowing in the desulphurizing media, such as limestone, soda, fluorspar, manganese and so forth, are known, and do not require further description.

It will be understood that our improved process may be carried out with various forms of apparatus and may be modified to suit varying conditions and requirements and we contemplate such changes and modifications as come within the spirit and scope of the appended claims.

We claim:

1. The process of manufacturing pig iron from

55

a burden rich in silica and using sulphur containing coke, characterized by the fact that in the lower part of the furnace, de-sulphurizing agents are blown into the charge, which contains slag-forming elements only in such quantities, that a high-sulphur iron would otherwise be produced together with an acid slag of low melting point.

5. The process of manufacturing pig iron from a burden rich in silica and using sulphur containing coke, characterized by the fact that in the lower part of the furnace, de-sulphurizing agents are blown into the charge, which contains slag-forming elements only in such quantities, that a high-sulphur iron would otherwise be produced together with an acid slag of low melting point, the pig iron being further desulphurized after tapping by means of additional desulphurizing reagents.

10. The process of manufacturing pig iron from a burden rich in silica and using sulphur containing coke, characterized by the fact that in the

lower part of the furnace, desulphurizing agents are blown into the charge, which contains slag-forming elements only in such quantities, that a high-sulphur iron would otherwise be produced together with an acid slag of low melting point, 5 the blowing-in of the desulphurizing agents in the lower part of the blast furnace being effected intermittently after withdrawal of the free-running silicious slag from the pig iron.

15. The process of manufacturing pig iron from a burden rich in sulphur and using sulphur containing coke, characterized by the fact that in the lower part of the furnace, desulphurizing agents are blown into the charge, which contains slag-forming elements only in such quantities 15 that a high-sulphur iron would otherwise be produced together with an acid slag of low melting point.

MAX PASCHKE.  
EUGEN PEETZ.

20